

[54] METHOD OF MANUFACTURING AN ARTICLE AND ARTICLE MANUFACTURED BY MEANS OF THE METHOD

[75] Inventor: **Hermanus Josephus Wilting**, Emmasingel, Eindhoven, Netherlands

[73] Assignee: **U.S. Philips Corporation**, New York, N.Y.

[22] Filed: **Dec. 7, 1972**

[21] Appl. No.: **312,847**

[30] Foreign Application Priority Data

Dec. 18, 1971 Netherlands ..... 7117429

[52] U.S. Cl. .... **117/212**, 156/5, 156/8,  
156/17

[51] Int. Cl. .... **B44d 1/18**, B21b 45/00

[58] Field of Search ..... 117/212, 217; 156/3, 7,  
156/17, 5, 8; 317/234 M

[56] References Cited

UNITED STATES PATENTS

3,686,080 8/1972 Banfield et al..... 117/212

Primary Examiner—John D. Welsh

Attorney, Agent, or Firm—Frank R. Trifari; Norman N. Spain

[57] ABSTRACT

The invention relates to the manufacture of a platinum pattern on a body, for example, for contacting a semiconductor body. First a layer of a material which can react with the platinum is provided on the body, namely in the form of a negative of the platinum pattern. A layer of platinum is then provided. The pattern of material is caused to react with the platinum layer and the reaction product of the material and the platinum is then removed after which the (positive) platinum pattern remains.

6 Claims, 5 Drawing Figures



Fig.1



Fig.2



Fig.3



Fig.4



Fig.5

METHOD OF MANUFACTURING AN ARTICLE  
AND ARTICLE MANUFACTURED BY MEANS OF  
THE METHOD

The invention relates to a method of manufacturing an article in which a platinum layer and a layer of a material which can react with the platinum are provided on a body, parts of the layer of material are removed so as to obtain a pattern of the material complementary to the desired platinum pattern, after which the platinum of the layer is caused to react with the material of the complementary pattern at elevated temperature and the reaction product of the material and the platinum is selectively removed relative to the platinum so as to obtain the platinum pattern, and to an article manufactured by means of the method.

The expression reaction to a reaction product is to be understood to mean herein not only the chemical reaction of the platinum with the material to form a chemical compound, but also, for example, the dissolving or alloying of the platinum and the material to form a product which can be selectively removed relative to the platinum. A pattern complementary to the platinum pattern is to be understood to mean herein a pattern which forms a negative relative to the platinum pattern as a positive pattern.

By means of this method, patterns can be obtained in platinum layers which cannot be realized, or be realized with difficulty, for example, by means of conventional photoetching methods.

The material may often be chosen to be such that the complementary pattern can be obtained in a usual manner, for example, photomechanically.

In a known method of the type mentioned in the preamble (see French Patent Specification No. 2,004,350) the complementary pattern of material is provided on the platinum layer and, after reaction of the material with the platinum layer, the reaction product is removed by etching as a result of which a (positive) platinum pattern remains.

In many applications, in which patterns are to be formed in platinum layers, not only a platinum layer is provided on the body in addition to the layer of material, but also layers of other metals, for example, chromium, titanium and/or gold, which in themselves can sometimes be etched better than platinum.

It is of advantage when all the metal layers including the layer of material, can be provided in one operation, for example, by vapour deposition.

The drawback is experienced that the material which is provided throughout the surface reacts with one or more metals differing from platinum already during the provision.

It is one of the objects of the invention to avoid the said drawback. The invention is inter alia based on the recognition of the fact that the last-mentioned reaction is prevented by providing the material in as early a stage as possible.

Therefore, the method mentioned in the preamble is characterized according to the invention in that first the complementary pattern of the material is provided on the body and then the platinum layer is provided.

It will be obvious that, since in the method according to the invention the material in the complementary pattern is first provided, the material can no longer react as the area of the desired pattern with after metal layers to be provided afterwards.

In the method according to the invention the material must of course be selectively removable relative to the body. As already stated above, the removal of the reaction product can be carried out by selective etching.

5 In a preferred embodiment of the method according to the invention, however, the reaction product is selectively removed relative to the platinum by means of an ultrasonic method. A reaction product often is much more brittle than the original platinum, as a result of 10 which mechanical methods of removing, for example, the ultrasonic method, is selective particularly in the method according to the invention.

Further it may be noted that combinations of the removal methods, such as etching and ultrasonic operation, are possible.

The material is preferably chosen from at least one element belonging to the group consisting of the elements of the groups IIIB and IVB of the periodic table.

20 In a variation of the method according to the invention the material chosen is germanium. A layer of titanium or chromium is preferably present between the layer of platinum and the body.

25 The invention furthermore relates to an article, in particular a semiconductor device, manufactured by means of the method according to the invention.

The invention will now be described in greater detail with reference to a drawing and a few examples.

FIGS. 1 to 5 are diagrammatic cross-sectional views 30 of a part of an article in successive stages of manufacture by means of the method according to the invention.

In the following example, a layer 2 of germanium is 35 provided on a silicon body 1 (FIG. 1). Germanium can react with platinum. Parts of the germanium layer 2 are removed so as to obtain a germanium pattern which is complementary to the desired platinum pattern (FIG. 2). A chromium layer 4 and a platinum layer 5 are then provided on the complementary germanium pattern (FIG. 3) and the platinum is caused to react with the 40 germanium to form a reaction product 6 (FIG. 4).

The reaction product 6 of the germanium and the platinum is selectively removed relative to the metal to obtain the platinum pattern (FIG. 5).

45 The germanium layer 2 is provided, for example, by vapour deposition and is approximately  $0.1 \mu$  thick.

The complementary germanium pattern is obtained in a usual manner by means of a photoetching method, in which a photolacquer layer is used as an etching mask for etching germanium in a bath containing hydrogen peroxide and, possibly, hydrofluoric acid.

The layers 4 and 5 are also provided by vapour deposition. The chromium layer is approximately 500 Å thick and the platinum layer 5 is approximately  $0.15 \mu$  thick. The temperature of the body 1 during the vapour deposition process is approximately  $450^\circ\text{C}$  the platinum diffusing through the thin chromium layer 4 and reacting with the underlying germanium. The reaction product of germanium and platinum is removed by dipping the body in aqua regia. The reaction product  $\text{GePt}_x$  dissolves in it many times faster than platinum alone. The reaction product may also be removed ultrasonically.

65 The chromium layer 4 serves to obtain a good adherence between the platinum layer 5 and the silicon body 1. With the said chromium layer 4, a reaction in the lateral direction is also prevented, as a result of which a

good edge sharpness of the platinum pattern is obtained.

With the layers 4 and 5 which need not everywhere adjoin directly the silicon but may be separated from it, for example, by an insulating oxide layer, regions of the silicon body can be contacted on the one hand, and on the other hand the platinum layer may be used for contacting connection conductors.

The platinum layer is preferably fortified with gold, for example, electrolytically, and titanium is used as an adhering layer instead of chromium. The contacting of a semiconductor body to obtain a semiconductor device may be carried out by:

- a. alloying a silicon body via apertures in an oxide layer with platinum;
- b. removing the non-reacted platinum on the oxide layer;
- c. vapour-depositing a germanium layer on the semiconductor body;
- d. providing the complementary pattern in the germanium layer;
- e. vapour-depositing a thin titanium layer, a platinum layer and a thin gold layer;
- f. reacting the metal layers with the germanium layer to form a reaction product;
- g. locally electrolytically thickening the gold layer;
- h. removing the reaction product. The reaction product may be etched away, but, owing to its brittle character, it may also be removed ultrasonically.

The method according to the invention is not restricted to the examples described but may be varied in many ways.

For example, the method is not restricted to the manufacture of semiconductor devices but in general arti-

cles may be manufactured having patterns, for example, for decorative applications.

Instead of germanium, the material used may be, for example, silicon, but also an element from the group 5 IIIB or IVB of the periodic table, for example, aluminum, may be used.

What is claimed is:

1. A method of providing a platinum pattern on a substrate said method comprising providing, in a pattern complementary to the desired platinum pattern, a layer of a material reactive with platinum on a substrate providing a layer of platinum on said material and on the exposed portions of the substrate, forming a reaction product of platinum and the material of the complementary pattern and selectively removing the reaction product of the platinum and the material from the body relative to the platinum thereby leaving the desired platinum pattern on the body.
- 10 2. A method as claimed in claim 1, wherein the reaction product is selectively removed relative to the platinum by means of ultrasonic energy.
- 15 3. A method as claimed in claim 1, wherein the material is chosen from at least one element belonging to the group consisting of the elements of groups IIIB and IVB 20 of the periodic table.
- 25 4. A method as claimed in claim 3, wherein the material chosen is germanium.
- 30 5. A method as claimed in claim 3, wherein a layer of titanium or chromium is present between the layer of platinum and the substrate.
- 35 6. A method as claimed in claim 1 wherein a layer of gold is provided on the platinum.

\* \* \* \* \*

35

40

45

50

55

60

65

UNITED STATES PATENT OFFICE  
CERTIFICATE OF CORRECTION

Patent No. 3,853,613

Dated December 10, 1974

Inventor(s) HERMANUS JOSEPHUS HENRICUS WILTING

It is certified that error appears in the above-identified patent  
and that said Letters Patent are hereby corrected as shown below:

In the title page, under "[75] Inventor:"

change "Hermanus Josephus Wilting" to  
-- Hermanus Josephus Henricus Wilting --.

Signed and Sealed this

*twenty-ninth* Day of July 1975

[SEAL]

Attest:

**RUTH C. MASON**  
Attesting Officer

**C. MARSHALL DANN**  
Commissioner of Patents and Trademarks